

3,301,667

PREPARATION OF URANIUM-NIOBIUM ALLOYS  
BY CO-REDUCTION

Waldo R. Gollerher and Robert A. Johnston, both of Paducah, Ky., assignors to the United States of America as represented by the United States Atomic Energy Commission

No Drawing. Filed Apr. 27, 1966, Ser. No. 546,479  
3 Claims. (Cl. 75—122.7)

The invention described herein was made in the course of, or under, a contract with the U.S. Atomic Energy Commission. The present invention relates to and has for its principal object the preparation of uranium-niobium alloys by bomb reduction in an essentially adiabatic process.

In order to produce an alloy of uranium by bomb reduction methods, a mixture of uranium tetrafluoride, a reducible salt or oxide of the alloying metal, and a co-reductant such as magnesium must be uniformly blended, packed into a refractory-lined container, and heated by external means until the reaction occurs. The resultant mass of metal that collects at the bottom of the lined cavity as one piece is known as a derby. The refractory lining and bomb container must meet several specifications to ensure good quality and yield of the alloy metal. These requirements are well-known to those skilled in the art. Briefly, it is that the refractory liner is primarily used to contain the alloy formed by the reaction and to protect the alloy from contamination by the bomb shell material. Since it comes in contact with the alloy formed, it must be relatively free of impurities that would unite with the alloy to impair its quality. After the liner is formed inside the bomb it must have sufficient green strength to have a charge packed into the resultant cavity without mixing with the charge. It must also have sufficient fired strength at the time of reaction to resist mixing with the reaction mass and thereby cause an inefficient separation of the metal and the slag produced by the reaction. One material that adequately meets this requirement is magnesium fluoride slag produced by the reaction as a by-product of  $UF_4$  by magnesium. An even more useful liner material is magnesia,  $MgO$ , because of its higher temperature stability and chemical inertness.

The initial source material for the metals of the alloys to be formed which can be used are limited to those which are reducible by a common reducing agent such as magnesium or mixture of calcium with iodine to effect total reduction of the respective source materials in a controllable and essentially adiabatic chemical reaction. The use of uranium tetrafluoride for chemical co-reductions of this type is well known and does not form a part of this invention per se. The essential and controlling choice is the niobium source material used in the co-reduction.

The salt of the metal chosen for the co-reduction with  $UF_4$  must be anhydrous, have a low vapor pressure at high temperatures near the reaction temperature with magnesium, and be available in sufficiently high purity so as not to grossly contaminate the resultant alloy with undesirable elements. Furthermore, it should be reducible in a reaction with magnesium or calcium that is not so highly reactive as to be dangerous. A still further requirement is that the alloy salt must be sufficiently stable up to a point of reaction so that it does not either inhibit the reaction or decompose prior to the desired reaction. Moreover, the fluoride reaction products of such a salt must not raise the melting point of the slag appreciably above the melting point of magnesium fluoride since this will adversely affect the fluidity of the slag and prevent adequate separation between the alloy and the slag.

It is the object of this invention to supply the foregoing

requirements by effecting an essentially adiabatic bomb co-reduction of a mixture of (1) uranium tetrafluoride and (2) a composition selected from either (a) a mixture of potassium fluoniobate and from 0-50%, by weight, based on the niobium of niobium pentoxide,  $Nb_2O_5$ , or (b) the reaction product resulting from a reaction between niobium pentafluoride and a fluoride salt selected from cesium fluoride, lithium fluoride, barium fluoride, calcium fluoride, uranyl fluoride, potassium fluoride, and magnesium fluoride.

The generic concept of this invention lies in the discovery that a particular class of selected niobium fluoride salt composition can be used in an essentially adiabatic co-reduction process of forming uranium-niobium alloys at a temperature much lower than is required for directly melting the respective elements of a desired alloy. What this invention provides is a reducible niobium salt as the initial niobium source which generates a heat of reaction with magnesium at least as great as that effected by the reduction of  $UF_4$  and magnesium to produce a low melting magnesium fluoride slag. This allows as much of a clean-cut slag-derby separation as is possible for such co-reductions while obtaining an alloy of desired composition. An ancillary concept of this development relates to the discovery that niobium pentafluoride, by itself a hygroscopic low melting compound, can be upgraded to a non-hygroscopic, high melting fluoride salt complex composition by reaction with the selected metal fluorides previously mentioned.

30 The selection of the proper niobium source material and success of the process lies in the recognition that the selected fluoride salts are stable and non-hygroscopic, as well as reducible under the same conditions required to reduce uranium tetrafluoride. Moreover, the secondary reaction product is, for the most part, magnesium fluoride which does not interfere with, or introduce any extraneous by-products which would tend to increase the melting point of the slag, or prevent its separation from the derby after it is formed.

40 Once the selected source materials are chosen to produce an alloy of desired composition, the efficiency of the co-reduction depends on the bomb firing conditions. With the reactants at room temperature, the heat of reaction is generally insufficient under adiabatic conditions to initiate and maintain the reduction products molten until an efficient separation has been effected between the mass of alloy derby and the resultant magnesium fluoride slag. Consequently, a resistance or induction-type furnace is used to initiate the reaction and to add the required heat to the reaction products to bring about an efficient separation between the alloy derby and the slag. Since the reactants are chosen to absorb the maximum possible heat, separation of the products will proceed most efficiently.

45 As a result, the firing schedule consists of preheating the mixture in the bomb at a low temperature such as 1300° F. for a period of time depending upon the quantity of heat required until the charge fires. In addition to the firing time, other variables that will influence the yield and quality of massive metal alloy derby from the reaction will include the reductant used, such as magnesium or calcium metal, or calcium mixed with a quantity of iodine; the melting point of the slag produced by the reaction and the melting point of the alloy itself to produce a sound substantially pure uranium-niobium alloy derby by reduction of  $UF_4$  and a selected niobium fluoride salt with magnesium. The optimum conditions are 7 to 10 stoichiometric excess of magnesium, 0-1% of the uranium as  $UO_2F_2$  with a furnace control temperature set at from 1200° F. to 1300° F. In terms of producing a high quality derby alloy in which quality is determined by size, weight, and shape of the derby, amount of voids, amount of slag

50

55

60

65

70

inclusions, and the degree to which the desired composition is realized, the preferred niobium salt is a mixture in which 50% of the niobium is obtained from  $\text{Nb}_2\text{O}_5$ , and the remainder from  $\text{K}_2\text{NbF}_7$ .

The following examples illustrate the method of co-reduction under essentially adiabatic conditions to produce a quality alloy derby in accordance with the general description previously provided.

### Example I

In this and the following examples the materials used were ingot magnesium supplied by the New England Lime Company,  $\text{UF}_4$  made by the reduction of  $\text{UF}_6$  with hydrogen, high purity —200 mesh niobium pentoxide, and —200 mesh potassium fluoniobate,  $\text{K}_2\text{NbF}_7$ , obtained from Kawecki Chemical Company. The co-reductions were made in steel bombs designed to produce a derby weight of about 4 kilograms. Magnesium fluoride liners were provided by jolting magnesium fluoride powder into the shell with a pneumatic mechanism. A globar resistance furnace was used to heat the bomb. The reduction bomb was instrumented with external thermocouples which indicated the bomb shell temperature at the bottom, middle, and top. A thermocouple was inserted into the charge to measure the temperature in the center of the charge.  $\text{UF}_4$  and other constituents of the bomb charge were thoroughly mixed in a V-type blender and charged into the magnesium fluoride lined shell. The charge was compacted and a magnesium fluoride liner was placed on top of it. A metal lid was then put in place and the bomb placed in a pre-heated furnace. The bomb temperatures were recorded and the time for the bomb to fire was noted. After the reaction was completed, the bomb was cooled and the contents were removed.

The following describes the subject process as used to produce a uranium-6 wt. percent niobium alloy derby.

4906 grams of  $\text{UF}_4$ , 54 grams of  $\text{UO}_2\text{F}_2$ , 393 grams of  $\text{K}_2\text{NbF}_7$ , and 172 grams of  $\text{Nb}_2\text{O}_5$  were thoroughly blended with 1008 grams of Mg, and the blend was charged into a  $\text{MgF}_2$ -lined steel reduction bomb sized to produce a 4-kg. uranium-derby. After the powder charge had been compacted and then capped with a layer of  $\text{MgF}_2$ , the bomb was closed with a steel lid and inserted in a resistance-heated furnace pre-heated to 1300° F. The bomb was instrumented to record its shell temperature and the temperature at the center of the charge. The following table summarizes this reduction run (indicated by an asterisk) as well as several related runs.

TABLE I

| Run No. | Nb as $\text{K}_2\text{NbF}_7\%$ <sup>1</sup> | Average Temp. at Firing, ° F. |         | Pre-ignition Time, Min. | Yield, Percent <sup>2</sup> |
|---------|-----------------------------------------------|-------------------------------|---------|-------------------------|-----------------------------|
|         |                                               | Center                        | Shell   |                         |                             |
| 1       | 0                                             |                               | 3,1,100 | 89                      | (4)                         |
| 2       | 0                                             | 875                           | 1,150   | 80                      | (4)                         |
| 3       | 50                                            | 1,225                         | 1,250   | 101                     | 99.8                        |
| 4       | *50                                           | 1,210                         | 1,225   | 93                      | 99.8                        |
| 5       | 75                                            | 1,125                         | 1,210   | 80                      | 100+                        |
| 6       | 75                                            | 1,060                         | 1,170   | 72                      | 93.5                        |
| 7       | 100                                           | 940                           | 1,150   | 72                      | 96.6                        |
| 8       | 100                                           | 950                           | 1,140   | 73                      | 100+                        |
| 9       | 100                                           | 900                           | 1,160   | 69                      | 99.9                        |

<sup>1</sup> The remainder of the niobium was added as  $\text{Nb}_2\text{O}_5$ .

<sup>2</sup> Contains some entrapped slag.

<sup>3</sup> Furnace pre-heated to 1200° F.

<sup>4</sup> No Derby.

The best quality derbies were obtained from runs 3-6 in which the niobium was provided in the form of at least 50%, by weight,  $\text{K}_2\text{NbF}_7$  with the remainder being niobium pentoxide. These derbies had a density approaching the theoretical density of the alloy composition but

contained numerous small voids and slight inclusions of incompletely separated slag. As the amount of  $\text{K}_2\text{NbF}_7$  increased to 100% the derbies contained increasingly larger voids and slag inclusions. Nevertheless, the derbies were of excellent quality and could readily be converted to a highly purified alloy ingot by a simple and straightforward melting operation for a time sufficient to allow separation of slag inclusions and removal of voids. A purified alloy casting is then obtained by bottom pouring into a casting mold. As shown in the table, no derby was formed when all of the niobium in the charge was present as  $\text{Nb}_2\text{O}_5$ .

### Example II

As previously mentioned, an ancillary generic concept of this invention is concerned with the provision of a unique class of stable complex niobium fluoride salts by reaction of the volatile, hygroscopic niobium pentafluoride,  $\text{NbF}_5$ , with selected stabilizing metal fluoride salts to produce a non-hygroscopic complex fluoride composition which is far more stable than niobium fluoride, wherein its stability depends on the relative amounts of the stabilizing metal fluoride additive. The several selected metal fluorides are dried in fluorine and then mixed at varying mole ratios with niobium pentafluoride in a dry atmosphere. Each mixture was placed in a nickel reactor. The reactor was then evacuated to a partial vacuum of about 0.1 millimeter mercury and heated to 400° F. for 4 hours to allow reaction to occur. After this, the reaction mixtures were cooled and the resulting compositions were determined on the basis of weight change and chemical analyses. The thermal stability of each material was determined by testing for weight changes using a thermobalance at temperatures ranging from 500-1400° F. The resultant data obtained is summarized in Table II.

TABLE II.— $\text{NbF}_5$ -METAL FLUORIDE COMPLEXES

| Run No. | Conditions          | $\text{CaF}_2$                   |                         |                                   |
|---------|---------------------|----------------------------------|-------------------------|-----------------------------------|
|         |                     | Composition                      | Time, <sup>1</sup> Hrs. | Approx. Decomposition Temp., ° F. |
| 50      | As Prepared         | 0.77 $\text{CaF}_2\text{-NbF}_5$ |                         | 300                               |
|         | Stable at 500° F.   | 1.24 $\text{CaF}_2\text{-NbF}_5$ | 7.4                     | 550                               |
|         | Stable at 800° F.   | 1.74 $\text{CaF}_2\text{-NbF}_5$ | 3.0                     | 900                               |
|         | Stable at 1,000° F. | 4.96 $\text{CaF}_2\text{-NbF}_5$ | 2.0                     | 1,275                             |
|         | Stable at 1,400° F. | 8.03 $\text{CaF}_2\text{-NbF}_5$ | 0.5                     |                                   |
| 55      | Conditions          | $\text{LiF}$                     |                         |                                   |
|         |                     | Composition                      | Time, <sup>1</sup> Hrs. | Approx. Decomposition Temp., ° F. |
|         | As Prepared         | 2.05 $\text{LiF}\text{-NbF}_5$   |                         | 500                               |
|         | Stable at 500° F.   | 2.20 $\text{LiF}\text{-NbF}_5$   | 0.5                     | 700                               |
|         | Stable at 800° F.   | 18.6 $\text{LiF}\text{-NbF}_5$   | 5.6                     | 950                               |
|         | Stable at 1,000° F. | 68.3 $\text{LiF}\text{-NbF}_5$   | 0.75                    | 1,100                             |
| 60      | As Prepared         | 2.05 $\text{LiF}\text{-NbF}_5$   |                         |                                   |
|         | Stable at 500° F.   | 2.20 $\text{LiF}\text{-NbF}_5$   | 0.5                     |                                   |
|         | Stable at 800° F.   | 18.6 $\text{LiF}\text{-NbF}_5$   | 5.6                     |                                   |
|         | Stable at 1,000° F. | 68.3 $\text{LiF}\text{-NbF}_5$   | 0.75                    |                                   |
|         | Stable at 1,400° F. | $\text{LiF}$ only                |                         |                                   |
|         |                     |                                  |                         |                                   |
| 65      | Conditions          | $\text{BaF}_2$                   |                         |                                   |
|         |                     | Composition                      | Time, <sup>1</sup> Hrs. | Approx. Decomposition Temp., ° F. |
|         | As Prepared         | 0.54 $\text{BaF}_2\text{-NbF}_5$ |                         | 300                               |
|         | Stable at 500° F.   | 0.55 $\text{BaF}_2\text{-NbF}_5$ | 0.2                     | 650                               |
|         | Stable at 800° F.   | 1.24 $\text{BaF}_2\text{-NbF}_5$ | 2.0                     | 900                               |
|         | Stable at 1,000° F. | 3.51 $\text{BaF}_2\text{-NbF}_5$ | 4.2                     | 1,100                             |
| 70      | As Prepared         | 0.54 $\text{BaF}_2\text{-NbF}_5$ |                         |                                   |
|         | Stable at 500° F.   | 0.55 $\text{BaF}_2\text{-NbF}_5$ | 0.2                     |                                   |
|         | Stable at 800° F.   | 1.24 $\text{BaF}_2\text{-NbF}_5$ | 2.0                     |                                   |
|         | Stable at 1,000° F. | 3.51 $\text{BaF}_2\text{-NbF}_5$ | 4.2                     |                                   |
|         | $\text{BaF}_2$ only | $\text{BaF}_2$ only              | 3.0                     |                                   |

TABLE II.—Continued

| Conditions              | UO <sub>2</sub> F <sub>2</sub> <sup>2</sup>                 |                            |                                             |
|-------------------------|-------------------------------------------------------------|----------------------------|---------------------------------------------|
|                         | Composition                                                 | Time, <sup>1</sup><br>Hrs. | Approx.<br>Decom-<br>position<br>Temp.,° F. |
| As Prepared.....        | 0.44 UO <sub>2</sub> F <sub>2</sub> -NbF <sub>5</sub> ..... |                            | 300                                         |
| Stable at 500° F.....   | 4.48 UO <sub>2</sub> F <sub>2</sub> -NbF <sub>5</sub> ..... | 0.5                        | 625                                         |
| Stable at 800° F.....   | 6.27 UO <sub>2</sub> F <sub>2</sub> -NbF <sub>5</sub> ..... | 0.3                        | 900                                         |
| Stable at 1,000° F..... | 6.71 UO <sub>2</sub> F <sub>2</sub> -NbF <sub>5</sub> ..... | 0.5                        | 1,100                                       |
| Stable at 1,400° F..... | UO <sub>2</sub> F <sub>2</sub> only.....                    | 2.0                        |                                             |

for an adiabatic co-reduction with uranium tetrafluoride to produce a desired uranium-niobium alloy.

*Example III*

5 This example illustrates the applicability of a complex double fluoride of niobium as prepared in Example II. Two complex fluoride compositions synthesized according to the procedure of Example II were mixed with appropriate amounts of uranium tetrafluoride and reduced in an adiabatic bomb reduction reaction as described in Example I. The results are tabulated in Table III below.

10 For purposes of comparison, runs 5 and 6 were conducted with the preferred niobium source (50-50 mixture

TABLE III

| Run No. | Percent Niobium Added As                |                                         |                                 |                                | Firing<br>Time<br>(Min.) | Derby<br>Density<br>(g./cc.) |
|---------|-----------------------------------------|-----------------------------------------|---------------------------------|--------------------------------|--------------------------|------------------------------|
|         | 0.87 BaF <sub>2</sub> -NbF <sub>5</sub> | 2.11 CaF <sub>2</sub> -NbF <sub>5</sub> | K <sub>2</sub> NbF <sub>7</sub> | Nb <sub>2</sub> O <sub>5</sub> |                          |                              |
| 1.....  | 63                                      |                                         |                                 |                                | 37                       | 14.2                         |
| 2.....  | 63                                      |                                         |                                 |                                | 37                       | 12.2                         |
| 3.....  | 63                                      |                                         |                                 |                                | 37                       | 12.3                         |
| 4.....  |                                         | 100                                     |                                 |                                | 62                       | 14.5                         |
| 5.....  |                                         |                                         | 50                              | 50                             | 50                       | 15.0                         |
| 6.....  |                                         |                                         | 50                              | 50                             | 50                       | 14.9                         |

| Conditions              | KF                             |                            |                                             |
|-------------------------|--------------------------------|----------------------------|---------------------------------------------|
|                         | Composition                    | Time, <sup>1</sup><br>Hrs. | Approx.<br>Decom-<br>position<br>Temp.,° F. |
| As Prepared.....        | 0.86 KF-NbF <sub>5</sub> ..... |                            | 150                                         |
| Stable at 500° F.....   | 1.21 KF-NbF <sub>5</sub> ..... | 2.4                        | 600                                         |
| Stable at 800° F.....   | 1.74 KF-NbF <sub>5</sub> ..... | 6.3                        | 950                                         |
| Stable at 1,000° F..... | 2.49 KF-NbF <sub>5</sub> ..... | 3.0                        | 1,100                                       |
| Stable at 1,400° F..... | 34.0 KF-NbF <sub>5</sub> ..... | 2.7                        |                                             |

| Conditions              | MgF <sub>2</sub>                              |                            |                                             |
|-------------------------|-----------------------------------------------|----------------------------|---------------------------------------------|
|                         | Composition                                   | Time, <sup>1</sup><br>Hrs. | Approx.<br>Decom-<br>position<br>Temp.,° F. |
| As Prepared.....        | 0.83 MgF <sub>2</sub> -NbF <sub>5</sub> ..... |                            | 200                                         |
| Stable at 500° F.....   | 0.86 MgF <sub>2</sub> -NbF <sub>5</sub> ..... | 0.7                        | 600                                         |
| Stable at 800° F.....   | 3.76 MgF <sub>2</sub> -NbF <sub>5</sub> ..... | 1.0                        | 900                                         |
| Stable at 1,000° F..... | 5.93 MgF <sub>2</sub> -NbF <sub>5</sub> ..... | 1.6                        | 1,100                                       |
| Stable at 1,400° F..... | 14.1 MgF <sub>2</sub> -NbF <sub>5</sub> ..... | 0.7                        |                                             |

<sup>1</sup> Approximate time to reach stable composition at temperature indicated in column 1.

<sup>2</sup> An attempt was also made to form UF<sub>4</sub>-NbF<sub>5</sub> complexes; none formed

As shown, each of the materials shown in the table is non-hygroscopic and has a thermal stability much higher than niobium pentafluoride, the thermal stability being a function of the selected metal fluoride to a niobium pentafluoride mole ratio. These compositions contain sufficient niobium to make them useful as source materials

25 of Nb<sub>2</sub>O<sub>5</sub>-K<sub>2</sub>NbF<sub>7</sub>). The differences are reflected in the derby density, a higher density indicating less porosity and/or slag inclusion. All derbies contained the pre-calculated alloy composition and can be melt casted to produce high purity alloy ingots.

30 Having thus described our invention, we claim:

1. A method for synthesizing a uranium-niobium alloy which comprises effecting an essentially adiabatic bomb co-reduction of a mixture of (1) uranium tetrafluoride and (2) a composition selected from either (a) a mixture of potassium fluoniobate and from 0-50%, by weight (based on the niobium of niobium pentoxide), Nb<sub>2</sub>O<sub>5</sub>, or (b) the reaction product resulting from a reaction between niobium pentafluoride and a fluoride salt selected from cesium fluoride, lithium fluoride, barium fluoride, calcium fluoride, uranyl fluoride, potassium fluoride, and magnesium fluoride.

35 2. The method according to claim 1 in which the source of niobium is derived equally from potassium fluoniobate and Nb<sub>2</sub>O<sub>5</sub>.

40 3. The method according to claim 1 in which 0-1% by weight of the uranium in the initial mixture is in the form of UO<sub>2</sub>F<sub>2</sub>, uranyl fluoride.

**References Cited by the Examiner**

50 Nuclear Science Abstracts, vol. 14, No. 10, May 31, 1960, Abstract No. 9713, p. 1234.

Reactor Core Materials, vol. 1, No. 2, May 1958, p. 4.

CARL D. QUARFORTH, Primary Examiner.

55 M. J. SCOLNICK, Assistant Examiner.